



US005290460A

**United States Patent** [19]**Habeeb et al.****[11] Patent Number:** **5,290,460****[45] Date of Patent:** **Mar. 1, 1994**

[54] **LUBRICANT COMPOSITION CONTAINING COMPLEXES OF ALKOXYLATED AMINE, TRITHIOCYANURIC ACID, AND ADENINE**

[75] **Inventors:** **Jacob J. Habeeb; Morton Beltzer,**  
both of Westfield, N.J.

[73] **Assignee:** **Exxon Research & Engineering Co.,**  
Florham Park, N.J.

[21] **Appl. No.:** **21,288**

[22] **Filed:** **Feb. 22, 1993**

[51] **Int. Cl.<sup>5</sup>** ..... **C10M 159/12; C10M 135/00;**  
**C07F 3/10**

[52] **U.S. Cl.** ..... **252/47.5; 544/277**

[58] **Field of Search** ..... **252/47.5; 544/277**

[56] **References Cited**

**U.S. PATENT DOCUMENTS**

|           |         |                  |       |            |
|-----------|---------|------------------|-------|------------|
| 3,156,689 | 11/1964 | Dexter et al.    | ..... | 260/248    |
| 3,198,797 | 8/1965  | Dexter et al.    | ..... | 260/249.5  |
| 3,202,681 | 8/1965  | Dexter et al.    | ..... | 260/249.5  |
| 3,255,191 | 6/1966  | Dexter et al.    | ..... | 260/248    |
| 3,334,046 | 8/1967  | Dexter et al.    | ..... | 252/47.5   |
| 3,723,428 | 3/1973  | Song             | ..... | 260/248 CS |
| 3,849,319 | 11/1974 | Nebzydoski       | ..... | 252/33.6   |
| 3,862,942 | 1/1975  | Gilles           | ..... | 260/248 CS |
| 3,951,973 | 4/1976  | Nebzydoski       | ..... | 260/248 CS |
| 4,038,197 | 7/1977  | Caspari          | ..... | 252/46.7   |
| 4,281,123 | 7/1981  | Hentschel et al. | ..... | 544/194    |
| 4,931,196 | 6/1990  | Payne et al.     | ..... | 252/47.5   |

**FOREIGN PATENT DOCUMENTS**

977589 12/1964 United Kingdom

*Primary Examiner*—Jerry D. Johnson  
*Attorney, Agent, or Firm*—James H. Takemoto

[57] **ABSTRACT**

A composition of matter useful in lubricating oil for reducing friction in an internal combustion engine, said complex comprising the reaction product of alkoxyLATED amine, trithiocyanuric acid and adenine and having the formula:



where R is a hydrocarbyl group of 2 to 22 carbon atoms, R<sup>1</sup> is hydrogen or a hydrocarbyl group of 1 to 20 carbon atoms, x and y are each independently integers of from 1 to 15 with the proviso that the sum of x+y is from 2 to 20, and a, b and c are independent numbers from 1.0 to 3.0 wherein the ratios between a:b, a:c and b:c range from 1.0:3.0 to 3.0:1.0.

**10 Claims, No Drawings**

**LUBRICANT COMPOSITION CONTAINING COMPLEXES OF ALKOXYLATED AMINE, TRITHIOCYANURIC ACID, AND ADENINE**

**BACKGROUND OF THE INVENTION**

**1. Field of the Invention**

This invention relates to the reaction product of alkoxylated amine, trithiocyanuric acid and adenine and to an improved lubricating oil composition containing the reaction product to reduce friction and improve fuel economy in an internal combustion engine.

**2. Description of the Related Art**

There are many instances, as is well known, particularly under "Boundary Lubrication" conditions where two rubbing surfaces must be lubricated, or otherwise protected, so as to prevent wear and to insure continued movement. Moreover, where, as in most cases, friction between the two surfaces will increase the power required to effect movement and where the movement is an integral part of an energy conversion system, it is most desirable to effect the lubrication in a manner which will minimize this friction. As is also well known, both wear and friction can be reduced, with various degrees of success, through the addition of a suitable additive or combination thereof, to a natural or synthetic lubricant. Similarly, continued movement can be insured, again with varying degrees of success, through the addition of one or more appropriate additives.

The primary oil additive for the past 40 years for providing antiwear and antioxidant properties has been zinc dialkyldithiophosphate (ZDDP). Oil formulations containing ZDDP, however, require friction modifiers in order to reduce energy losses in overcoming friction. Such energy losses result in lower fuel economy. Moreover, oil additive packages containing ZDDP have environmental drawbacks. ZDDP adds to engine deposits which can lead to increased oil consumption and emissions. Moreover, ZDDP is not ash-free. Various ashless oil additive packages have been developed recently due to such environmental concerns.

U.S. Pat. Nos. 3,849,319 and 3,951,973 describe lubricant compositions containing di- and tri(hydrocarbylammonium)trithiocyanurates. The hydrocarbyl radicals include alkyl, aralkyl, aryl, alkaryl and cycloalkyl and the examples are directed to alkylamines. These lubricant compositions were stated to have improved load-carrying properties.

It would be desirable to have a lubricating oil composition which provides excellent friction reducing, fuel economy properties and environmentally beneficial (less fuel, i.e., less exhaust emission) properties.

**SUMMARY OF THE INVENTION**

This invention relates to a novel composition of matter containing alkoxylated amine, trithiocyanuric acid, and adenine and to an improved lubricating oil composition which reduces friction and improves fuel economy in an internal combustion engine as well as provides copper corrosion inhibition. The composition of matter comprises the reaction product of alkoxylated amine, thiocyanuric acid and adenine wherein said reaction product is a complex having the formula



where R is a hydrocarbyl group of 2 to 22 carbon atoms, R¹ is hydrogen or a hydrocarbyl group of 1 to 20 carbon atoms, x and y are each independently integers of from 1 to 15 with the proviso that the sum of x+y is from 2 to 20, and a, b and c are independent numbers from 1.0 to 3.0 wherein the ratios of a:b, a:c and b:c range from 1.0:3.0 to 3.0:1.0. In another embodiment, there is provided a lubricant composition comprising a major amount of a lubricating oil basestock and a minor amount of a complex having the formula (I). Yet another embodiment relates to a method for reducing friction in an internal combustion engine which comprises operating the engine with a lubricating composition containing an amount effective to reduce friction of a complex having the formula (I) set forth above.

**DETAILED DESCRIPTION OF THE INVENTION**

In the lubricating oil composition of the present invention, the lubricating oil will contain a major amount of a lubricating oil basestock. The lubricating oil basestock are well known in the art and can be derived from natural lubricating oils, synthetic lubricating oils, or mixtures thereof. In general, the lubricating oil basestock will have a kinematic viscosity ranging from about 5 to about 10,000 cSt at 40° C., although typical applications will require an oil having a viscosity ranging from about 10 to about 1,000 cSt at 40° C.

Natural lubricating oils include animal oils, vegetable oils (e.g., castor oil and lard oil), petroleum oils, mineral oils, and oils derived from coal and shale.

Synthetic oils include hydrocarbon oils and halo-substituted hydrocarbon oils such as polymerized and interpolymerized olefins, alkylbenzenes, polyphenyls, alkylated diphenyl ethers, alkylated diphenyl sulfides, as well as their derivatives, analogs, and homologs thereof, and the like. Synthetic lubricating oils also include alkylene oxide polymers, interpolymers, copolymers and derivatives thereof wherein the terminal hydroxyl groups have been modified by esterification, etherification, etc. Another suitable class of synthetic lubricating oils comprises the esters of dicarboxylic acids with a variety of alcohols. Esters useful as synthetic oils also include those made from C<sub>5</sub> to C<sub>12</sub> monocarboxylic acids and polyols and polyol ethers.

Silicon-based oils (such as the polyalkyl-, polyaryl-, polyalkoxy-, or polyaryloxy-siloxane oils and silicate oils) comprise another useful class of synthetic lubricating oils. Other synthetic lubricating oils include liquid esters of phosphorus-containing acids, polymeric tetrahydrofurans, polyalphaolefins, and the like.

The lubricating oil may be derived from unrefined, refined, rerefining oils, or mixtures thereof. Unrefined oils are obtained directly from a natural source or synthetic source (e.g., coal, shale, or tar sands bitumen) without further purification or treatment. Examples of

unrefined oils include a shale oil obtained directly from a retorting operation, a petroleum oil obtained directly from distillation, or an ester oil obtained directly from an esterification process, each of which is then used without further treatment. Refined oils are similar to the unrefined oils except that refined oils have been treated in one or more purification steps to improve one or more properties. Suitable purification techniques include distillation, hydrotreating, dewaxing, solvent extraction, acid or base extraction, filtration, and percolation, all of which are known to those skilled in the art. Rerefined oils are obtained by treating refined oils in processes similar to those used to obtain the refined oils. These rerefined oils are also known as reclaimed or reprocessed oils and often are additionally processed by techniques for removal of spent additives and oil breakdown products.

In the oil soluble complexes of the present invention having the formula (I), R is preferably a hydrocarbyl group of from 2 to 18 carbon atoms, especially 6 to 18 carbon atoms, and R<sup>1</sup> is preferably hydrogen or a hydrocarbyl group of from 1 to 16 carbon atoms, most preferably hydrogen. Such hydrocarbyl groups include aliphatic (alkyl or alkenyl) and alicyclic groups. The aliphatic or alicyclic groups may be substituted with 23 amino, hydroxy, mercapto and the like and may be interrupted by O, S or N. The sum of x+y is preferably 2 to 15.

The complexes of the present invention are prepared from the reaction of alkoxylated, preferably ethoxylated, especially ethoxylated amines with trithiocyanuric acid and adenine. Adenines are commercially available or may be prepared by methods known in the art. Ethoxylated and/or propoxylated amines are commercially available from Sherex Chemicals under the trade name Varonic and from Akzo Corporation under the trade names Ethomeen®, Ethoduomeen® and Propomeen®. Examples of preferred amines include ethoxylated (5) cocoalkylamine, ethoxylated (2) tallowalkylamine, ethoxylated (15) cocoalkylamine and ethoxylated (5) soyaalkylamine.

Trithiocyanuric acid may exist in different tautomeric forms represented by formulas II, III or mixtures thereof:



Trithiocyanuric acid is prepared by methods well known in the art. These methods involve the treatment of cyanuric chloride with sulfur nucleophiles according to the following reaction schemes:



-continued



10 Other sulfur nucleophiles which may be employed in the above reaction scheme include sodium sulfide, thio-urea and thioacetic acid

The complexes according to the invention are prepared by adding trithiocyanuric acid to a mixture of adenine and alkoxylated amine. Because of the exothermic nature of the reaction, the reaction mixture should be stirred during addition of trithiocyanuric acid. The amounts of reactants are approximately stoichiometric, although a slight excess of trithiocyanuric acid, which has three reactive hydrogens, may be employed.

The precise stoichiometry of the bonding in the complexes of the formula (I) is not known since each molecule in the complex may have several sites which can take part in the hydrogen bonding process either as an acceptor or donor. Because of the multiplicity of bonding possibilities, the molar ratios  $a:b:c$  can be varied over a wide range based on the donor/acceptor sites on each of the three molecules and therefore  $a$ ,  $b$  and  $c$  in formula (I) are numbers which are not necessarily integral. There exist a total of forty-five combinations of interaction sites between the three molecules comprising the complex of the formula (I). For example,  $a:b:c$  may be 1:2:1 or 1:1:3 which are just two of the forty-five possible combinations.

The lubricant oil composition according to the invention comprises a major amount of lubricating oil base-  
40 stock and an amount effective to increase fuel economy of the alkoxylated amine:trithiocyanuric acid:adenine complex. Typically, the amount of complex will be from about 0.001 wt % to about 5 wt %, based on oil  
45 basestock. Preferably, the amount of amine salt is from about 0.05 wt % to about 1.0 wt %.

If desired, other additives known in the art may be added to the lubricating oil basestock. Such additives include dispersants, antiwear agents, antioxidants, rust inhibitors, other corrosion inhibitors, detergents, pour point depressants, extreme pressure additives, viscosity index improvers, other friction modifiers, hydrolytic stabilizers and the like. These additives are typically disclosed, for example, in "Lubricant Additives" by C. V. Smalhear and R. Kennedy Smith, 1967, pp. 1-11 and in U.S. Pat. No. 4,105,571, the disclosures of which are incorporated herein by reference.

The lubricating oil composition of this invention can be used in the lubrication system of essentially any internal combustion engine, including automobile and truck engines, two-cycle engines, aviation piston engines, marine and railroad engines, and the like. Also contemplated are lubricating oils for gas-fired engines, alcohol (e.g., methanol) powered engines, stationary powered engines, turbines, and the like.

This invention may be further understood by reference to the following example, which includes a preferred embodiment of this invention.

## EXAMPLE 1

This Example illustrates the preparation of a complex containing ethoxylated amine, trithiocyanuric acid and adenine according to the invention. 68 g of ethoxylated(5)cocoalkylamine and 13 g of adenine was heated to 70° C. with stirring in a 3-neck round bottom flask fitted with a thermometer and a water cooled condenser. 14 g of trithiocyanuric acid was added gradually to the stirred amine solution. During addition, the temperature rose to 105° C. due to an exothermic reaction between acid and amine adenine components. The reaction mixture was used without further purification.

## EXAMPLE 2

The complex containing ethoxylated amine, trithiocyanuric acid and adenine is an effective friction modifier as shown in this example. The Ball on Cylinder (BOC) friction tests were performed using the experimental procedure described by S. Jahanmir and M. Beltzer in ASLE Transactions, Vol. 29, No. 3, p. 425 (1985) using a force of 0.8 Newtons (1 Kg) applied to a 12.5 mm steel ball in contact with a rotating steel cylinder that has a 43.9 mm diameter. The cylinder rotates inside a cup containing a sufficient quantity of lubricating oil to cover 2 mm of the bottom of the cylinder. The cylinder was rotated at 0.25 RPM. The friction force was continuously monitored by means of a load transducer. In the tests conducted, friction coefficients attained steady state values after 7 to 10 turns of the cylinder. Friction experiments were conducted with an oil temperature of 100° C. Various amounts of the complex prepared in Example 1 were added to solvent 150N. The results of BOC friction tests are shown in Table 1.

TABLE 1

| Wt % of Ethoxylated (5) Cocoalkylamine, Adenine, Trithiocyanuric Acid Complex in Solvent 150N* | Coefficient Of Friction |
|------------------------------------------------------------------------------------------------|-------------------------|
| 0.00                                                                                           | 0.29                    |
| 0.05                                                                                           | 0.06                    |
| 0.1                                                                                            | 0.05                    |
| 0.2                                                                                            | 0.05                    |
| 0.3                                                                                            | 0.05                    |
| 0.5                                                                                            | 0.025                   |
| 0.8                                                                                            | 0.025                   |
| 1.0                                                                                            | 0.010                   |

\*S150 is a solvent extracted, dewaxed, hydrofinned neutral lube base stock obtained from approved paraffinic crudes (viscosity, 32 cSt at 40° C., 150 Saybolt seconds)

As can be seen from the results in Table 1, as little as 50 0.05 wt % of complex shows 79% decrease in the coefficient of friction. These results demonstrate that present complexes are capable of significant reductions in the coefficient of friction of a lubricant basestock which results in less friction and hence greater fuel economy 55 when the lubricated oil is used in an internal combustion engine.

What is claimed is:

1. A composition of matter comprising a complex which is the reaction product of alkoxyated amine, 60 trithiocyanuric acid and adenine, said complex having the formula



where R is a hydrocarbyl group of 2 to 22 carbon atoms, R<sup>1</sup> is hydrogen or a hydrocarbyl group of 1 to 20 carbon atoms, x and y are each independently integers of from 1 to 15 with the proviso that the sum of x+y is from 2 to 20, and a, b and c are independent numbers from 1.0 to 3.0 wherein the ratios between a:b, a:c and b:c range from 1.0:3.0 to 3.0:1.0.

- 15 2. The composition of claim 1 wherein R is alkyl or alkenyl of 2 to 18 carbon atoms.
- 20 3. The composition of claim 1 wherein the sum of x+y is 2 to 15.
- 25 4. The composition of claim 1 wherein R<sup>1</sup> is hydrogen.
5. A lubricant oil composition comprising
- (a) a major amount of a lubricating oil basestock, and
- (b) a minor amount of a complex comprising the reaction product of alkoxyated amine, trithiocyanuric acid and adenine, said complex having the formula



where R is a hydrocarbyl group of 2 to 22 carbon atoms, R<sup>1</sup> is hydrogen or a hydrocarbyl group of 1 to 20 carbon atoms, x and y are each independently integers of from 1 to 15 with the proviso that the sum of x+y is from 2 to 20, and a, b and c are independent numbers from 1.0 to 3.0 wherein the ratios between a:b, a:c and b:c range from 1.0:3.0 to 3.0:1.0.

6. The composition of claim 5 wherein R is alkyl or alkenyl of 2 to 18 carbon atoms.
7. The composition of claim 5 wherein the sum of x+y is 2 to 15.
8. The composition of claim 5 wherein R is hydrogen.
9. The composition of claim 5 wherein the amount of complex is from about 0.001 wt. % to about 5 wt. %, based on oil.

10. A method for reducing friction in an internal combustion engine which comprises operating the engine with the lubricating oil composition of claim 5.

\* \* \* \* \*